

# UNITED STATES PATENT OFFICE.

GEORGE DIEFFENBACH, OF NEW YORK, N. Y.

## IMPROVEMENT IN BASES FOR ARTIFICIAL TEETH.

Specification forming part of Letters Patent No. 19,916, dated April 13, 1858.

*To all whom it may concern:*

Be it known that I, GEORGE DIEFFENBACH, of the city, county, and State of New York, have invented a new and Improved Base for Artificial Teeth; and I do hereby declare that the following is a full, clear, and exact description of my invention and of its application.

The substances at present in use, or the use of which has been attempted, for the purpose of forming a base for artificial teeth are metals, ivory, hippopotamus, and gutta-percha. My experience in dentistry having shown to me the serious disadvantages consequent upon the use of the said materials for the said purpose, I deem it necessary in the first place to detail these injurious effects as follows:

First. All metals being good conductors of heat, cause a disagreeable sensation of chill in the mouth by their rapid absorption of its natural heat.

Second. The perpetual contact of every metal with parts of the mouth causes a disagreeable taste, an unnatural excitement of the glands, an increased secretion of the saliva, and with some persons a weakening of the nervous system.

Third. Most of the metals oxidize by the action of the stomach-acid. Platina is an exception to this rule; but its great weight makes its retention in the mouth a matter of great difficulty.

Fourth. The proper shape of a metallic base for artificial teeth not being obtainable by a direct process, is inexact in many cases, and its retention in the mouth, as well as its service in chewing, is thereby rendered extremely difficult.

Fifth. All metals used for this purpose are liable to bend and to lose their original shape by a continued use in the mouth.

Sixth. Ivory, hippopotamus, and gutta-percha are injuriously effected by the saliva, they frequently require renewals, and emit, moreover, a disagreeable odor.

These defects have induced me to invent a composition of matter which may be worn in the mouth without being liable to any of the injurious effects above enumerated. The idea soon suggested itself to me that amber was free from all these defects; but I found it too brittle to be formed into the proper shapes. I have therefore endeavored by an extended se-

ries of observations and experiments to form a composition of matter in which amber was to be the principal ingredient, and which could be cast or molded into the various shapes necessary for the base of artificial teeth; and, my efforts having become successful, I will here state that the nature of my invention consists in forming a proper base for artificial teeth of a composition of matter containing amber as its most prominent ingredient.

To enable others skilled in the art to make and use my invention, I will proceed to describe its composition and application.

I pulverize amber and put the same in a crucible (the inside of which ought to be glazed) over a soft-coal fire, the intensity of which is gradually increased until the amber begins to melt, when it is agitated until the whole of the pulverized amber is molten. I then take linseed-oil and pour the same while in a boiling state into the molten amber and agitate the mixture. I then remove it from the fire, but continue to stir it until it becomes cool. In this state the composition, although less brittle than pure amber, does not possess the tenacity requisite for my purpose. I therefore add purified pulverized sulphur, and mix the whole well together. I then put the same in an iron retort, and apply heat to the same until the whole mass is gradually hardened. I deem it proper to state that I have found steam heat the most advantageous for my purpose, and that bringing the retort in direct contact with the fire somewhat injures the result; and I will further remark that I have varied the proportions of these ingredients, but I have found the following to be sufficiently accurate for my purpose: I take to one pound of amber, one-half pound of prepared linseed-oil, and two ounces of sulphur. I have named linseed-oil and sulphur because they are the cheapest substances known to me to effect the desired end. Caoutchouc may be added in small quantities without impairing the result; but I do not claim such addition as any part of my invention. I am also enabled to impart to the above-described composition any color that may be deemed desirable by the admixture of proper pigments during the process of preparation. I use this composition to form the following parts of the mouth, namely: the gum, the alveola, (maxilla inferior,) the palate,

(maxilla superior,) and the jaw—thus acquiring a complete base for artificial teeth.

I make these articles in the following manner: I take an impression in wax or in plaster-of-paris of that part of the mouth which I wish to imitate. I then pour fluid plaster into that impression (with the usual precaution for separation) and leave it therein until dry. Thereby I obtain the original mold. I then arrange and fasten the requisite number of artificial teeth on this mold, which is now ready to receive the hot composition, consisting of amber, linseed-oil, gutta-percha, and sulphur, as above described. This is now put into the model and its thickness regulated as desired. I then put the plaster model, with its contents, into the retort above described, leaving it there until fully hardened. When removed the artificial base is complete in form and in substance.

It will be seen that I obtain my ultimate form direct from the original mold, (whereas the use of metals requires the original mold to be formed in sand and cast in a metal which has to be recast in a softer metal, called the "female" mold, which is separated from the other, and the sheet metal for the base is put between the two molds and hammered or stamped between them.)

The great usefulness of this invention for dental purposes, and its superiority over the existing methods of forming a base for artificial teeth, consists in the following points:

First. The amber composition is tasteless, it causes no excitement of the glands, it creates an agreeable feeling in the mouth, and emits no odor.

Second. The contact between the amber composition and the mouth is not injurious to health and acts as preventive against some diseases—such as inflammation of the throat, &c.

Third. Being a bad conductor of heat, it does not cause sudden feelings of cold in the mouth.

Fourth. It is not liable to oxidation, corrosion, or solution by the action of the stomach-acid or the saliva.

Fifth. It is capable of bearing extreme degrees of heat and cold without suffering any injury therefrom.

Sixth. It can be easily cast into any shape suitable to the mouth, it is not liable to bend, it always retains its form, and for these reasons it affords great security for its retention in the mouth and increased facility in chewing.

Seventh. Being enabled to firmly unite the artificial teeth with this composition without the use of any other cement or solder, by uniting them before the composition becomes hardened I obtain a compact body and avoid pores between the teeth and their base.

Eighth. It is cheaper than most of the metals.

What I claim as new, and desire to secure by Letters Patent, is—

Making the base for artificial teeth of a composition of matter in which amber forms the principal ingredient, in the manner substantially as described.

New York, December 10, 1857.

GEORGE DIEFFENBACH.

Witnesses:

CHS. WEHLE,  
JOHN MOODY.